

Dec. 17, 1946.

H. CRAWSHAW

2,412,562

FABRIC

Filed June 27, 1944

FIG. 1



FIG. 2



FIG. 3



Inventor  
H. CRAWSHAW

By  
I. Seltzer & C. Lebowitz  
Attorneys

## UNITED STATES PATENT OFFICE

2,412,562

## FABRIC

Harry Crawshaw, London, England, assignor to  
 British Celanese Limited, London, England, a  
 company of Great Britain

Application June 27, 1944, Serial No. 542,386  
 In Great Britain May 21, 1943

5 Claims. (Cl. 139—425)

1

This invention relates to fabrics. For certain purposes, e. g. for the interception of radio waves, there is a demand for a strong, light-weight, flexible fabric which is a good conductor of electricity. This combination of properties is not easily obtained by any of the prior methods of wire-fabric construction. Plain-woven wire fabrics in which successive wires in both warp and weft are widely spaced apart to give the desired flexibility and lightness, and to provide the desired electrical conductivity without excessive consumption of wire, are unsatisfactory since the wires tend to slip over one another and also do not make sufficiently tight contact to give the desired conductivity. Wire fabrics having a true gauze structure are very difficult to weave owing to the extent to which the wire warps must be distorted to produce such a structure.

I have now found that a fabric having the desired properties can be obtained by weaving a fabric in which, in both warp and weft, narrow bands of fine wires alternate with broad bands of textile yarns, at least two warp wires being interlaced with at least two weft wires at each crossing of the wire bands of warp and weft. Preferably the ratio of the total area of the spaces between the wires to the product of the diameter of the wire and the length of wire is not less than about 10:1.

It is sometimes desirable e. g. when the fabric is to be used in the construction of kites, drogues or pilotless aircraft, which are required to be capable of intercepting radio-signals, for the fabric to be of low wind-resistance. Fabrics having this property can be obtained from the wire-textile yarn fabrics described above by removing the textile yarn locally or throughout. This can be done, e. g. by means of an agent which dissolves or otherwise destroys the yarn without affecting the wire. When an open-mesh, all-wire fabric is made in this way, i. e. by weaving a wire-textile yarn fabric of the structure specified above and subsequently removing the textile yarn, the textile yarns serve to space apart and locate the wires during weaving; they enable a tight beat-up to be obtained and assist in kinking the wires at the crossings so that they slip less easily over one another. By local removal of the textile yarns from a wire-textile yarn fabric of the structure specified, an open-work electrically conducting fabric can be obtained, in which in certain areas, e. g. round the margin of the fabric, panels filled with interwoven textile yarns remain to facilitate attachment of the

2

fabric to other fabrics or materials, e. g. by sewing.

The following examples illustrate the invention.

5

*Example 1*

On a two-box loom a fabric of the following construction is woven.

Weave: plain.

10 Warp: 48 pairs of yarns each pair woven as one (about 100 pairs to the inch), each yarn of 30 denier regenerated cellulose yarn of high tenacity, alternating with two pairs of wires each pair woven as one end, each wire of 40 British standard wire gauge tinned-copper wire.

15 Weft: 24 single picks (about 100 to the inch) each of the regenerated cellulose yarn specified above, alternating with two single picks, each of the wire specified above.

The structure of this fabric is shown in Figs. 1  
 20 and 2 of the accompanying diagrammatic drawings wherein Fig. 1 is a plan-view on a much enlarged scale of a small portion of the fabric and Fig. 2 is a plan-view on a smaller scale of a larger portion of the same fabric.

25 Referring now to Fig. 1, the pairs of warp yarns 10 are each composed of two identical yarns 11. The pairs of wires 12 are each composed of two identical wires 13. The weft is composed of a number of single picks of textile yarn 14 alternating with two picks 15 of wire.

The fabric when viewed as a whole appears to consist, as shown in Fig. 2, of rectangular panels 16 of interwoven textile yarn each panel being about twice as long as it is broad, and 35 being bounded along the two long sides by narrow bands 18 of wire and along the two shorter sides by wider bands 17 of wire.

This fabric may be used as such as an electrical screening fabric, or as a material for picking up or transmitting radio waves. The fabric may be used in the construction of kites intended to intercept or transmit radio signals.

*Example 2*

45 A fabric is woven as described in Example 1 but substituting for the regenerated cellulose yarn a yarn of high tenacity cellulose acetate, made by stretching a cellulose acetate yarn of normal tenacity to many times its original length in steam or hot water.

The panels of interwoven cellulose acetate yarn are removed except along the margin of the fabric, by applying acetone locally to the fabric. This may be done by means of a brush, or the 55 marginal portions may be coated with a resist

for acetone, which can subsequently be removed without damaging the cellulose acetate in the said marginal portions, and the fabric may then be given an overall treatment, e. g. in a bath, with acetone to remove the unreserved panels.

A portion of fabric so treated is shown diagrammatically in plan-view in Fig. 3, where a central area in which the cellulose acetate has been removed leaving spaces 19 between the bands of wires, is bounded by a marginal area in which the cellulose acetate panels 18 have remained intact. A fabric of this kind is specially suitable for the construction of kites and the like since by virtue of the large spaces between the bands of wires it has low windage whereas the marginal panels of cellulose acetate yarns enable lengths of the fabric to be sewn together or otherwise attached to one another or to other materials.

The fabric described in Example 1 can be 20 treated as described in Example 2 but substituting for acetone a solvent for regenerated cellulose, e. g. cuprammonium sulphate or ammonium thiocyanate.

Various modifications can be made in the structure of the wire-textile yarns without departing from the principle of construction outlined above, viz: that of employing in both warp and weft narrow bands of wires alternating with broad bands of textile yarn, at least two warp wires and at least two weft wires being interlaced at each crossing of the wire bands of warp and weft. Thus, for example, instead of employing pairs of similarly shedded wires in the warp of the fabric described above, single yarns and wires can be 35 employed although better results qua flexibility, conductivity and freedom from slip are obtained using the pairs of ends. The bands of wire in warp and weft may also contain more wires than those of the fabric described, provided that the bands of wire remain sufficiently narrow relative to the bands of textile yarn to give the desired open texture in the final wire fabric. Thus, for example, the weft bands may consist of more than two single picks, for example 4 or 6 single 40 picks may be employed (odd numbers of wires in the weft bands are preferably avoided as involving complication in the loom); or two wires may be inserted at each pick. The principle of construction referred to could be applied in the production of fabrics other than plain woven fabrics, for example twill fabrics, but the best combination of properties has been obtained using a plain weave and especially a construction of the kind specifically described above.

A measure of the spacing apart of the bands of wire of the wire-fabrics or wire-textile yarn fabrics of the invention, in the initial wire-textile fabrics, is given by the ratio: total area of spaces between wires to product of diameter of wire by length of wire. This ratio may vary between wide limits, e. g. from less than 8:1 to over 50:1. In the preferred form of the invention the ratio is between about 10:1 and about 20:1, e. g. about 12:1.

The ratio: total area of spaces between wire bands to area occupied by the wire bands should not be less than about 4:1 and is preferably considerably higher, e. g. between about 6 or 8:1 and about 16:1 or even higher. A useful figure for this ratio using wires of about 0.005" in diameter is about 8:1.

Tinned copper wire has been found the most satisfactory material for the conductive element of the fabric but other ductile metals of good

electrical conductivity could be employed, for example aluminium. When high electrical conductivity is not of importance metals of lower conductivity than aluminium can be used, e. g. iron. The diameter of the wire employed may range from less than 0.005" up to 0.01" or even higher, e. g. above 0.02".

The high-tenacity regenerated cellulose yarn referred to above, may be made by the saponification of a cellulose acetate yarn which has been stretched to many times its original length under the influence of steam, hot water or an organic stretch-assisting agent. Such regenerated cellulose yarns may have a tenacity considerably greater than two grams per denier, for example 3-4, 5 or 6 grams per denier or even higher. High tenacity in the textile material which is interwoven with the wire in carrying out the present invention is of considerable advantage in enabling a strong, tightly-woven fabric to be obtained. Other textile materials can be employed, however, in the place of regenerated cellulose of the kind referred to. Among such other materials are regenerated cellulose yarn made by the viscose or cuprammonium processes; yarn having a basis of an organic derivative of cellulose, for example cellulose acetate, cellulose propionate, cellulose acetate-propionate, cellulose acetate-butyrate, ethyl cellulose and benzyl cellulose; 25 yarn having a basis of a polymerised unsaturated substance or substances, for example polystyrene, polyethylacrylate, polymethyl methacrylate, polyvinyl acetate, polyvinyl chloride, polyvinyl chloride-acetate and polyvinylidene chloride; and 30 yarn composed of artificial fibres of a proteinaceous substance such as casein or soya bean protein. Yarns of natural textile fibre, for example cotton, linen, silk or wool can also be employed. The textile material selected should be in the 35 form of strong, fine filaments. When it is intended to produce an open-work fabric by removal of the textile yarn, this yarn should, of course, be capable of destruction by agents which will not damage the wire. Regenerated cellulose 40 yarns obtained by the saponification of highly-stretched cellulose acetate yarns are particularly suitable in all these respects. Other of the textile fibres referred to above can be employed with 45 advantage in the form of yarns having a high tenacity. For instance high tenacity yarns of any 50 of the cellulose derivatives specified may be used.

The nature of the agent employed to disintegrate the textile material will of course depend on the nature of that material. For materials of natural or regenerated cellulose, excellent results have been obtained with cuprammonium sulphate. Other agents capable of disintegrating these materials are strong mineral acids, e. g. hydrochloric acid, capable of effecting rapid hydrolysis of cellulose, and salts, for example the alkali metal thiocyanates, capable of dissolving cellulose. In the case of natural and artificial textile materials having a proteinaceous basis, strong alkalies will usually be found effective. 55 For cellulose derivatives and polymerised unsaturated fibre-forming substances appropriate organic solvents can be found, for example, in the case of cellulose acetate, acetone can be employed. In selecting an agent for disintegrating the textile material, agents which would damage the wire will of course be avoided.

Having described my invention, what I desire to secure by Letters Patent is:

1. A woven fabric suitable for intercepting 60 radio signals, said fabric having in both warp

and weft narrow bands of fine copper wire, at least two warp wires being interlaced with at least two weft wires at each crossing of the wire bands of warp and weft, in any sample the ratio of the total area of the spaces between the wires to the product of the diameter of the wire and the length of the wire in said sample being not less than about 8:1, and the spaces enclosed by the bands of wires being filled with interwoven non-metallic textile yarns.

2. A woven fabric suitable for intercepting radio signals, said fabric having in both warp and weft narrow bands of fine copper wire, at least two warp wires being interlaced with at least two weft wires at each crossing of the wire bands of warp and weft, in any sample the ratio of the total area of the spaces between the wires to the product of the diameter of the wire and the length of the wire in said sample being between about 10:1 and about 20:1, and the spaces enclosed by the bands of wires being filled with interwoven non-metallic textile yarns.

3. A woven fabric suitable for intercepting radio signals, said fabric having in both warp and weft narrow bands of fine copper wire, at least two warp wires being interlaced with at least two weft wires at each crossing of the wire bands of warp and weft, in any sample the ratio of the total area of the spaces between the wires to the product of the diameter of the wire and the length of the wire in said sample being between about 10:1 and about 20:1, and the spaces

enclosed by the bands of wires being filled with interwoven regenerated cellulose yarns of tenacity at least 4 grams per denier.

4. A woven fabric suitable for intercepting radio signals, said fabric having in both warp and weft narrow bands of fine copper wire, at least two warp wires being interlaced with at least two weft wires at each crossing of the wire bands of warp and weft, in any sample the ratio of the total area of the spaces between the wires to the product of the diameter of the wire and the length of the wire in said sample being between about 10:1 and about 20:1, the spaces enclosed by the bands of wires being filled with interwoven non-metallic textile yarns and each of said spaces being of area about  $\frac{1}{8}$  square inch.

5. A woven fabric suitable for intercepting radio signals, said fabric having in both warp and weft narrow bands of fine copper wire, at least two warp wires being interlaced with at least two weft wires at each crossing of the wire bands of warp and weft, in any sample the ratio of the total area of the spaces between the wires to the product of the diameter of the wire and the length of the wire in said sample being between about 10:1 and about 20:1, the spaces enclosed by the bands of wires being filled with interwoven regenerated cellulose yarns of tenacity at least 4 grams per denier and each of said spaces being of area about  $\frac{1}{8}$  square inch.

HARRY CRAWSHAW.